

# United States Patent [19]

Ho

[11] Patent Number: 4,902,404

[45] Date of Patent: Feb. 20, 1990

[54] HYDROTREATING PROCESS WITH  
CATALYST STAGING

[75] Inventor: Teh C. Ho, Baton Rouge, La.

[73] Assignee: Exxon Research and Engineering  
Company, Florham Park, N.J.

[21] Appl. No.: 215,093

[22] Filed: Jul. 5, 1988

[51] Int. Cl.<sup>4</sup> ..... C10G 45/08; C10G 47/04

[52] U.S. Cl. ..... 208/57; 208/254 H;  
208/228; 208/249

[58] Field of Search ..... 208/57, 58, 216 R, 254 H,  
208/217, 246, 247, 249, 303, 228

[56] References Cited

U.S. PATENT DOCUMENTS

- |           |        |                 |             |
|-----------|--------|-----------------|-------------|
| 3,459,656 | 8/1969 | Rausch          | 208/57      |
| 3,594,307 | 7/1971 | Kirk, Jr.       | 208/57      |
| 4,022,682 | 5/1977 | Bludis et al.   | 208/254 H X |
| 4,243,553 | 1/1981 | Naumann et al.  | 502/220     |
| 4,528,089 | 7/1985 | Pecoraro et al. | 208/254 H X |

4,591,429 5/1986 Ho et al. .... 208/254 H  
4,650,503 3/1987 Jacobson et al. .... 208/254 H X  
4,698,145 10/1987 Ho et al. .... 208/254 H X  
4,705,619 11/1987 McCandish et al. .... 208/254 H

Primary Examiner—Glenn Calderola  
Attorney, Agent, or Firm—Henry E. Naylor

[57] ABSTRACT

Disclosed is a process for hydrotreating a hydrocarbonaceous feed wherein the feed is treated with hydrogen, at hydrotreating conditions, in a first catalyst zone containing a conventional hydrotreating catalyst. The treated feed is then further treated in a second catalyst zone containing a catalyst represented  $MM'_aS_x$  where M is Cr or one or more divalent promoter metals selected from Mn, Fe, Co, Ni, Cu, and Zn; M' is one or both of Mo and W; x is 0.5 to 9, and a=1 when Cr is not one of metals represented by M, and  $1 < a \leq 1.5$  when Cr is one of the metals represented by M.

7 Claims, No Drawings

## HYDROTREATING PROCESS WITH CATALYST STAGING

### FIELD OF THE INVENTION

The present invention relates to a staged hydrotreating process in which two or more catalyst zones are employed. The first, or upstream, zone contains a conventional supported catalyst while the second, or downstream, zone contains a sulfide catalyst derived from metal amine molybdates (or tungstates) or metal amine thiomolybdates (or thiotungstates).

### BACKGROUND AND PROBLEMS

Hydrotreating of petroleum feedstocks and various boiling fractions thereof, has become increasingly important because of more stringent product quality requirements. Furthermore, the petroleum industry foresees the time when it will have to turn to relatively high boiling feeds derived from such materials as coal, tar sands, oil-shale, and heavy crudes. Feeds derived from such materials generally contain significantly more deleterious components, such as sulfur, nitrogen, oxygen, halides, and metals. Consequently, such feeds require a considerable amount of upgrading in order to reduce the content of such components, thereby making them more suitable for further processing, such as fluid catalytic cracking and/or catalytic reforming.

Hydrotreating is well known in the art and usually requires treating a hydrocarbonaceous feed with hydrogen, in the presence of a catalyst to effect conversion of at least a portion of the feed to lower boiling products, and/or removal of deleterious components. See for example U.S. Pat. No. 2,914,462 which discloses the use of molybdenum sulfide for hydrodesulfurizing gas oil and U.S. Pat. No. 3,148,135 which discloses the use of molybdenum sulfide for hydrorefining sulfur and nitrogen-containing hydrocarbon oils. Further, U.S. Pat. No. 2,715,603 discloses the use of molybdenum sulfide as a catalyst for the hydrogenation of heavy oils, while U.S. Pat. No. 3,074,783 discloses the use of molybdenum sulfides for producing sulfur-free hydrogen and carbon dioxide, wherein the molybdenum sulfide converts carbonyl sulfide to hydrogen sulfide. Molybdenum and tungsten sulfides have other uses as catalysts, including hydrogenation, methanation, water gas shift, etc. reactions.

In general, with molybdenum and other transition metal sulfide catalysts, as well as with other types of catalysts, greater catalyst surface areas generally result in more active catalysts than similar catalysts with lower surface areas. Thus, those skilled in the art are constantly trying to achieve catalysts having ever greater surface areas. More recently, it has been disclosed in U.S. Pat. Nos. 4,243,553 and 4,243,554 that molybdenum sulfide catalysts of relatively high surface area may be obtained by thermally decomposing selected thiomolybdate salts at temperatures ranging from about 300°-800° C. in the presence of essentially inert, oxygen-free atmospheres. Suitable atmospheres are disclosed as consisting of argon, a vacuum, nitrogen, and hydrogen. In U.S. Pat. No. 4,243,554, an ammonium thiomolybdate salt is decomposed at a rate in excess of 15° C. per minute, whereas in U.S. Pat. No. 4,243,553, a substituted ammonium thiomolybdate salt is thermally decomposed at substantially slower heating rate of about 0.5 to 2° C./min. The processes disclosed in these patents are claimed to produce molybdenum disulfide

catalysts having superior properties for water gas shift and methanation reactions as well as for catalyzed hydrogenation and hydrotreating reactions.

Hydrotreating catalysts comprising molybdenum sulfide, in combination with other metal sulfides, are also known. For example, U.S. Pat. No. 2,891,003 discloses an iron-chromium composition for desulfurizing olefinic gasoline fractions. Further, U.S. Pat. No. 3,116,234 discloses Cr-Mo and also Mo with Fe and/or Cr and/or Ni for hydrodesulfurization. Also U.S. Pat. No. 3,265,615 discloses Cr-Mo for hydrodenitrogenation and hydrodesulfurization.

Hydrotreating catalysts can also be used in a multi-stage process or in a stacked-bed process. For instance, U.S. Pat. No. 4,392,945 discloses a hydrodesulfurization process by using a two-stage reactor system with inter-stage removal of H<sub>2</sub>S and NH<sub>3</sub>. The first stage reactor contains a Ni-promoted conventional catalyst, while the second stage reactor contains a Co-promoted conventional catalyst. U.S. Pat. No. 4,534,852 discloses a stacked-bed process. The catalyst in the upstream zone contains phosphorus in the range of 2-4 wt% and is a Ni-promoted Mo sulfide catalyst. The catalyst in the downstream zone has a phosphorus level of less than 0.5 wt% and is an Mo sulfide catalyst promoted by Co and/or Ni. Both catalysts are supported on a carrier consisting mostly of alumina and are prepared via conventional techniques. This stacked-bed process is primarily applicable to resids hydrotreating wherein catalyst deactivation by metals and coke is a primary process concern.

More recently, new classes of hydrotreating catalysts have been developed which comprise self-promoted molybdenum and/or tungsten sulfide. For example, U.S. Pat. No. 4,663,023, which is incorporated herein by reference, teaches the catalysts represented by the formula MM'A<sub>x</sub> where M is one or more promoter metals such as Ni and Co; M' is Mo and/or W; x is a number 1 to 5, and A is oxygen or sulfur. These catalysts are prepared from a precursor represented by ML(M<sub>y</sub>W<sub>1-y</sub>A<sub>4</sub>) wherein M is one or more promoter metals, L is one or more, neutral, nitrogen-containing ligands at least one of which is a chelating polydentate ligand; and y is any value from 0 to 1, and A is O or S. These precursors are also taught in U.S. Pat. No. 4,595,676, which is also incorporated herein by reference. Other precursors and taught in U.S. Pat. Nos. 4,591,429; 4,632,747; and 4,668,376 all of which are incorporated herein by reference. Further, chromium-molybdenum and tungsten sulfide catalysts are taught in U.S. Pat. Nos. 4,622,128; 4,626,339; and 4,716,139, all of which are also incorporated herein by reference.

### SUMMARY OF THE INVENTION

In accordance with the present invention, there is provided an improved hydrotreating process, which process comprises:

(a) contacting the feed in a first catalyst zone at a temperature from about 200° C. to about 450° C., in the presence of hydrogen wherein the catalyst is comprised of at least one metal selected from Group VIB and at least one metal selected from Group VIII of the Periodic Table of the Elements, on an inorganic oxide support material; and

(b) contacting the treated feedstream from said first catalyst zone in a second catalyst zone at a temperature from about 200° C. to about 450° C., in the presence of

hydrogen wherein the catalyst in the second catalyst zone can be formally represented by the formula  $MM'_aS_x$  where M is Cr and/or one or more divalent promoter metals selected from the group consisting of Mn, Fe, Co, Ni, Cu, and Zn; M' is one or both of Mo and W; x is within the range of  $0.5 \leq x \leq 9$ . When none of the metals represented by M is Cr,  $a=1$ . When one of the metals represented by M is Cr,  $1 \leq a \leq 1.5$ , wherein said catalyst is derived from a precursor selected from the formula:



where M is Cr, and/or one or more divalent promoter metals selected from the group consisting of Mn, Fe, Co, Ni, Cu, and Zn; L is one or more neutral, nitrogen-containing ligands at least one of which is a chelating polydentate ligand;  $0 \leq y \leq 1$ ; A is O or S; and a is as defined above.

The Cr-containing catalysts can also be prepared from a mixture of (1) a hydrated oxide of trivalent chromium and (2) a salt containing a thiometallate anion of Mo or W and a cation comprising at least one divalent promoter metal chelated by at least one neutral, nitrogen-containing polydentate ligand. In this case, a is within the range of  $0.5 \leq a \leq 3$  and more preferably within the range of  $0.8 \leq a \leq 2$ .

#### DETAILED DESCRIPTION OF THE INVENTION

A variety of feedstocks can be hydrotreated in accordance with the present invention including both hydrocarbon fractions and whole feeds. Non-limiting examples of such feeds include organic solvents, light, middle and heavy distillates, and residual feeds.

In practicing hydrotreating in accordance with the present invention, a sulfur and/or nitrogen containing feedstream is contacted with hydrogen in a first catalyst stage, or zone, at hydrotreating conditions with a catalyst composition comprised of active metal components and an inorganic refractory support, preferably an inorganic oxide. The active metal component is comprised of at least one metal from Group VIB of the Periodic Table of the Elements and at least one promoter metal, preferably a metal from Group VIII of the Periodic Table of the Elements, on an inorganic oxide support. Preferred Group VIB metals are molybdenum and tungsten. More preferred is molybdenum. Preferred Group VIII metals are selected from cobalt, nickel, and iron. More preferred are cobalt and nickel. The amounts of active metal components range from about 0.5 to 20 wt. %, preferably from about 1 to 8 wt. %, more preferably from about 2 to 5 percent wt. %, in terms of its oxide, based on the total weight of the catalyst for the Group VIII metal, and from about 5 to 30 wt. %, preferably from about 8 to 25 wt. %, and more preferably from about 12 to 20 wt. %, in terms of an oxide, based on the total weight of the catalyst for the Group VIB metal. Support materials suitable for use herein are any conventional support material used in the manufacture of hydrotreating catalysts. Such materials are usually refractory oxides of elements of Groups II to IV of the Periodic Table of the Elements. The Periodic Table to which all of the Groups herein refer to can be found on the last page of *Advanced Inorganic Chemistry*, 2nd Edition, 1966, Interscience Publishers, by Cotton and Wilkenson. Preferred are alumina, silica, and silica-alumina. More preferred is alumina. The alumina may contain up to 5 wt. % of silica or phosphate to stabilize

it and/or to give the required pore characteristics. An alumina support means, therefore, one with at least 99 wt. % alumina.

It is understood that one or more catalyst zones, or 5 stages, can be contained in one or more reactors, but it is preferred to have two catalyst zones stacked in a single reactor. Such an arrangement is sometimes referred to as a stacked-bed reactor.

The feedstock, after being treated in the first zone, is 10 contacted with hydrogen at hydrotreating conditions in a second catalyst zone. The catalyst in the second zone is comprised of a catalyst formally represented by the formula  $MM'_aS_x$  where M is Cr and/or one or more divalent promoter metals selected from the group consisting of Mn, Fe, Co, Ni, Cu, and Zn; M' is one or both of Mo and W; x is a number from 0.5 to 9 and more preferably from 1 to 5;  $a=1$  when Cr is not one of the metals represented by M and  $0.5 < a \leq 3$  or more preferably  $0.8 \leq a \leq 2$  when Cr is one of the metals represented by M, with or without another promoter metal. The catalysts can be derived from two types of precursors. In one case, the catalyst is derived from a precursor represented by  $ML(Mo_yW_{1-y}A_4)_a$  where M is as defined above; L is one or more neutral, nitrogen-containing ligands at least one of which is a chelating polydentate ligand;  $0 \leq y \leq 1$ ; A is O or S and a is defined as above.

Preferably, M will be selected from the group consisting of: (a) Ni, Co, Fe and mixtures thereof, and (b) mixtures of (a) with Zn, Cu, Mn, Cr. Still more preferably M will be selected from the group consisting of Fe, Mn, Ni, Co, Cr and mixtures thereof. Thus, the promoter metal may be a single metal such as Ni, in which case the precursor will have the formula  $(NiL)(Mo_yW_{1-y}A_4)$ . Alternatively the promoter metal may be a mixture of two, three, four, five, or even six promoter metals. For the case of two promoter metals, such as Ni and Co, the precursor will have the formula  $[(Ni_bCo_{1-b})L](Mo_yW_{1-y}A_4)$  where  $0 < b < 1$ , and so on for the case where 3, 4, 5 or 6 promoter metals are present. The precursor may be a self promoted molybdate, thiomolybdate, tungstate, thiotungstate or combination thereof. If it is a molybdate, then y will have a value of 1. Alternatively, if the precursor is tungstate, y will be zero.

In the other case, which is applicable to only the Cr-containing catalysts, the catalyst is derived from a mixture of (i) a hydrated oxide of trivalent chromium and (ii) a thiometallate salt of the general formula  $ML(Mo_yW_{1-y}S_4)$  wherein M is one or more divalent promoter metals selected from the group consisting of Ni, Co, Mn, Cu, Zn, mixtures thereof, and mixtures thereof with Fe, wherein y is any value ranging from 0 to 1 and L is one or more neutral, nitrogen-containing ligands at least one of which is a chelating polydentate ligand. The total denticity of the ligands used to form the precursor compound will be about six.

If desired, more molybdenum and/or tungsten sulfide 60 may be incorporated into the precursor, and concomitantly the composition of this invention, by also including in the precursor mixture a thiometallate salt of the general formula  $(L')(Mo_yW_{1-y}S_4)$  wherein y is as above and L' is the conjugate acid of one or more ligands, L, with a charge sufficient to balance the negative charge of the thiometallate anion. In such a case the precursor will comprise a mixture of (i) a hydrated oxide of trivalent chromium, (ii) a thiometallate salt

containing the desired divalent promoter metal of the formula  $(ML)Mo_yW_{1-y}S_4$  and (iii) a thiometallate salt of the formula  $(L')(Mo_yW_{1-y}S_4)$ .

The ligand L, will generally have a denticity of six and will be one or more neutral, nitrogen-containing ligands wherein at least one of said ligands, is a multi-dentate chelating ligand which chelates the promoter metal to form a chelated promoter metal cation  $[ML]^{2+}$ . Thus, the catalytic metal oxide anion  $(Mo_yW_{1-y}A)^{2-}$  will be ionically bound to the chelated promoter metal cation  $[ML]^{2+}$ . By neutral is meant that the ligand itself does not have a charge.

Those skilled in the art know that the term "ligand" is used to designate functional coordinating groups which have one or more pairs of electrons available for the formation of coordinate bonds. Ligands that can form more than one bond with a metal ion are called polydentate while ligands that can form only one bond with a metal ion are called monodentate. Monodentate ligands are not capable of forming chelates. Hence, if one uses one or more species of monodentate ligands in the precursor molecule, then one must also use at least one polydentate chelating ligand. Preferably, L will be one or more polydentate chelating ligands. The denticity of the ligand L will generally be six, because the promoter metal cationss prefer six-fold coordination. Hence, if more than one species of ligand is employed in the precursor molecule, the denticity of the ligand species will usually add up to six. It should be understood that it is possible for ligand L to have a total denticity of less than six, but in most cases L will have a total denticity of six. Thus, L will be three bidentate ligands, two tridentate ligands, a mixture of a bidentate and a quadrentate ligand, a hexadentate ligand or a mixture of a polydentate ligand with monodentate ligands, as long as the combination has a total denticity of six. As has heretofore been stated, it is preferred to use chelating bidentate and tridentate ligands. In general, the ligands useful in this invention include alkyl and aryl amines and nitrogen heterocycles. Illustrative, but non-limiting examples of ligands useful in the catalyst precursors of this invention are set forth below.

Monodentate ligands will include  $NH_3$ , as well as alkyl and aryl amines such as ethyl amine, dimethyl amines, pyridine, etc. Useful chelatoing bidentate amine ligands are illustrated by ethylenediamine, 2,2'-bipyridine, 1,10-phenylene bis(dimethyl-amine), o-phenylene diamine, tetramethylethylenediamine and propane-1,3 diamine. Similarly, useful chelating tridentate amine ligands are represented by terpyridine and diethylenetriamine while triethylenetetramine is illustrative of a useful chelating quadradentate amine ligand. Useful chelating pentadentate ligands include tetraethylenepenetramine while sepolchrate (an octazacryptate) is illustrative of a suitable chelating hexadentate ligand. However, as a practical matter it will be preferred to use chelating, polydentate alkyl amines for L. Illustrative, but not limiting examples of alkyl amines that are useful in the catalyst precursor of this invention include ethylenediamine, diethylenetriamine, and tetraethylenetetramine. It is particularly preferred to use bidentate and tridentate alkyl amines such as ethylenediamine and diethylenetriamine.

In general, the precursor salts useful for forming the catalysts of this invention and which are represented by the aforementioned formula when M is not Cr, may be prepared by mixing an aqueous solution of ammonium molybdate and/or tungstate for A=oxygen and am-

nium thiomolybdate and/or thiotungstate for A=sulfur, with an aqueous solution of chelated promoter metal cation, for example,  $[ML]^{2+}$  which, in the presence of excess metallate (A=O), or thiometallate (A=S), ligand and/or chelated promoter metal cation, will result in the formation of the precursor salt as a precipitate which is readily recovered. The chelating promoter cation is easily formed by, for example, mixing an aqueous solution of one or more water soluble promoter metal salts with the ligand or mixture of ligands. The water soluble salt may be any water soluble salt that is convenient to use. Non-limiting examples of such salts include halides, sulfates, perchlorates, acetates, nitrates, etc. Alternatively, an aqueous solution of ammonium molybdate and/or tungstate, or ammonium thiomolybdate and/or thiotungstate may be mixed with the ligand with the resulting solution mixed with an aqueous solution of promoter metal salt. The salt can also be added to the ligand and dissolved into the solution of molybdate and/or tungstate or thiomolybdate and/or thiotungstate, as the case may be. It should be understood that the catalyst precursor preparation is not intended to be limited to aqueous media.

When the composition of the present invention can contain chromium, two different procedures can be used for the precursor preparation. In one procedure, the chromium containing precursor is prepared by mixing a slurry of (i) a hydrated oxide of trivalent chromium  $Cr(OH)_3 \cdot xH_2O$ , with (ii) one or more of the promoter metal and ligand containing thiometallate salts and, optionally, (iii) one or more thiometallate salts of Mo and/or W containing the conjugate acid of one or more ligands, but no divalent promoter metal. The thiometallate salt is then precipitated onto the slurried particles of hydrated chromium oxide and the precursor is recovered. The hydrated chromium oxide may be freshly precipitated from an aqueous solution of a trivalent chromium salt. Alternatively, the source of hydrated chromic oxide may be a colloidal, aqueous suspension of same. In one method of preparation the hydrated chromium oxide will be precipitated from an aqueous solution of trivalent chromium salt by contacting said salt solution with one or more basic amine chelating agents.

In one embodiment, a water soluble trivalent chromium compound and divalent metal salt are dissolved in water and hydrated chromium oxide is precipitated by addition of a ligand, L, or a mixture of ligands, L. This procedure produces a slurry or suspension of very fine particles of a hydrated oxide of trivalent chromium in the aqueous phase, which also contains some free ligand L, and some of the conjugate acid of the ligand L, L'. When the conjugate acid is a strong acid, that is, if the ligand L is a weak base, then a quantity of ammonium hydroxide may be added to precipitate the chromium. The water soluble chromium salt may be any water soluble salt that is convenient to use such as halide, sulfate, nitrate, etc. Sufficient ligand L is added to form the water soluble chelated promoter metal cations  $[ML]^{2+}$ . This suspension of hydrated chromium oxide containing  $[ML]^{2+}$  in solution is then mixed with a solution of the thiometallate prepared by dissolving ammonium thiometallate in an excess of the ligand or mixture of ligands. A small amount of water may be added if desired. On mixing the slurry with the thiometallate solution, an orange-red colored precipitate of the catalyst precursor forms which is recovered by filtration. This precipitate will be a precursor of a composi-

tion of this invention. Any step of this preparation may be done in the presence of a slurry of support material. If the chromia is present in sufficient amount, then the excess will serve as all or a portion of the support.

In another embodiment the thiometallate salts (ML)Mo<sub>y</sub>W<sub>1-y</sub>S<sub>4</sub>) and (L')(Mo<sub>y</sub>W<sub>1-y</sub>S<sub>4</sub>) may be prepared separately and mixed separately or together with the hydrated chromium oxide slurry prepared as described above. Again, this may be done in the presence of a slurry of support material. If the chromia is present in sufficient amount, then the excess chromia will comprise all or a portion of the support.

The salts (L')(Mo<sub>y</sub>W<sub>1-y</sub>S<sub>4</sub>) may generally be prepared by dissolving the ammonium thiometallate in excess of the ligand L. The salt is recovered as a precipitate by addition of water or some other suitable antisolvent such as methanol or acetone. If desired, these salts may be formed in the presence of one or more precursor materials as well as in the presence of one or more support materials. This procedure and precursor have more fully been discussed in U.S. Pat. No. 4,622,128 which is incorporated herein by reference.

The chromium-containing precursor compositions can also be prepared by mixing a solution of an appropriate thiometallate such as ammonium thiomolybdate and/or thiotungstate in a mixture of ligand(s) L and water with an aqueous solution of the chelated promoter metal cation, containing trivalent chromium [Cr<sub>1-z</sub>M<sub>z</sub>L<sub>y</sub>]<sup>2n+</sup>, which results in the formation of the precursor compound as a precipitate which is readily recovered. The chelated, trivalent chromium containing cation is formed under anhydrous conditions by dissolving a soluble salt of trivalent chromium, such as CrCl<sub>3</sub>, in an appropriate ligand or ligand mixture at low temperature (i.e., 0° C.). When this solution is warmed up to ambient temperature, the chelating reaction occurs and the chelated salt precipitates. The product can be filtered, washed with methanol and dried for subsequent use. The chelated divalent metal promoter cation is easily formed by, for example, mixing an aqueous solution of one or more water soluble promoter metal salts with the ligand. The water soluble salt may be any water soluble salt that is convenient to use such as a halide, sulfate, perchlorate, acetate, nitrate, etc. While the chelated salts are generally water soluble, they can be precipitated from their aqueous solutions by the addition of methanol, filtered and washed with methanol, and dried. For example, solid Ni(en)<sub>3</sub>Cl<sub>2</sub> can be prepared by adding ethylenediamine (en) to an aqueous solution of NiCl<sub>2</sub>·6H<sub>2</sub>O, adding methanol to precipitate the chelate, washing with methanol and drying.

The anhydrously prepared chelated chromium cation salt is dissolved in water along with the chelated divalent promoter salt. The ammonium thiometallate solution is mixed with this solution containing the chelated promoters, resulting in the precipitation of the catalyst precursor. This procedure and precursor are more fully discussed in U.S. Pat. No. 4,716,139 which is incorporated herein by reference.

The difference in the method of preparing the chelated chromium promoter cation from the chelated divalent metal promoter cations is the fact that chromium chelation is slow compared to that of the divalent ions. As a result, the addition of the basic ligand to an aqueous chromium salt solution will result in the formation predominantly of hydrated chromium oxide instead of the chelate (CrL)Cl<sub>3</sub>. To avoid this hydrated oxide formation, the chromium chelation is carried out under

anhydrous conditions by adding the trivalent chromium salt to the dry ligand. One can prepare the divalent promoter metal chelates in the same manner, either separately or along with the trivalent chromium chelates.

The catalysts contained in the downstream catalyst zone may be used in bulk or they can be on a suitable support. It is preferred that they be dispersed on an inorganic oxide such as alumina. As previously stated, an advantage of the catalyst precursors where A=oxygen resides in their water solubility which permits them to be supported on suitable support materials by techniques well-known in the art, such as impregnation, incipient wetness, and the like. The choice is left to the convenience of the practitioner. When using the impregnation technique, the aqueous impregnating solution will be contacted with the support for a time sufficient to deposit the precursor material onto the support either by selective adsorption or alternatively, the excess water may be evaporated during drying, leaving behind the precursor salt. Advantageously, an incipient wetness technique may be used whereby just enough of an aqueous precursor salt solution is added to dampen and fill the pores of the support. Where A=S and it is desired that the catalyst contains a support material, the precursor salt preparation may be done in the presence of a slurry of support material, in which case the precursor salt will be formed or precipitated onto the surface of the support material. Alternatively, the precursor salt or salts may be prepared and then composited with support material to form the catalyst precursor composite.

Prior to use, the catalysts of this second zone are presulfided by heating one or more catalyst precursor salts, bulk or supported, in the presence of sulfur in a non-oxidizing atmosphere, at a temperature of at least about 200° C. for a time sufficient to form the catalyst. Preferably, the sulfur required during the formation of the catalyst will be present in the form of a sulfur bearing compound and in amount in excess of that required to form the catalyst. Thus, it is preferred that the catalyst be formed by heating the precursor in the presence of sulfur or, preferably in the presence of a sulfur bearing compound which can be one or more solids, liquids, gases or mixtures thereof. Mixtures of hydrogen and H<sub>2</sub>S have been found to be particularly preferred. Preferably, the temperature will range between from about 250°-600° C., more preferably from about 250°-500° C. and still more preferably from about 300°-450° C. The non-oxidizing atmosphere may be inert or net reducing.

As discussed above, molybdenum and tungsten sulfide catalysts have many uses, including hydrotreating. Hydrotreating conditions vary considerably depending on the nature of the hydrocarbon being hydrotreated, the nature of the impurities or contaminants to be reacted or removed, and, inter alia, the extent of conversion desired, if any. In general, however, the following are typical conditions for hydrotreating a naphtha boiling within a range of from about 25° C. to about 210° C., a diesel fuel boiling within a range of from about 170° C. to 350° C., a heavy gas oil boiling within a range of from about 325° C. to about 475° C., a lube oil feed boiling within a range of from about 290°-500° C., or residuum containing from about 10 percent to about 50 percent of material boiling above about 575° C.

## Catalyst Sulfiding

| Feed     | Temp., °C. | Pressure psig | Space Velocity V/V/Hr. | Hydrogen Gas Rate SCF/B |
|----------|------------|---------------|------------------------|-------------------------|
| Naphtha  | 100-370    | 150-800       | 0.5-10                 | 100-2000                |
| Diesel   | 200-400    | 250-1500      | 0.5-6                  | 500-6000                |
| Heavy    | 260-430    | 250-2500      | 0.3-4                  | 1000-6000               |
| Lube Oil | 200-450    | 100-3000      | 0.2-5                  | 100-10,000              |
| Residuum | 340-450    | 1000-5000     | 0.1-2                  | 2000-10,000             |

The following examples are presented to illustrate the invention.

## Feedstock

Two feedstocks were used in the examples to be discussed later. Feedstock A is a light catalytic cycle oil (LCCO). Feedstock B is a virgin distillate. The properties of these feedstocks are set forth in Table 1 below.

TABLE I

| Properties of Feedstocks A and B |             |             |
|----------------------------------|-------------|-------------|
|                                  | Feedstock A | Feedstock B |
| API Gravity at 60° F.            | 16.5        | 32.9        |
| Sulfur, Wt. %                    | 1.35        | 0.37        |
| Nitrogen, WPPM                   | 715         | 92          |

## Equipment/Procedure

The evaluation experiments were conducted in a fixed-bed reactor immersed in a sand bath. The reactor was packed with about 10 cc of catalyst(s) in the central zone and denstone in the fore and aft zones. To ensure an adequate reactor-to-particle diameter ratio, the catalysts were crushed into 14/35 mesh granules. To obtain the lined-out activity, the reaction under a particular set of conditions was allowed to proceed for at least 24 hours before the first product sample was analyzed. The liquid product was analyzed for total sulfur by X-ray fluorescence and for nitrogen by combustion analysis. Test conditions were 330 psig, 625° F., 1500 SCF/B H<sub>2</sub>, and 1.0 LHSV.

## Data Analysis/Results

The following mass balance equation for a second-order reaction occurring in a plug-flow reactor is used to determine volumetric rate constant for HDS, K<sub>HDS</sub>.

$$K_{HDS} = LHSV \left( \frac{1}{S_p} - \frac{1}{S_f} \right)$$

wherein S<sub>f</sub> and S<sub>p</sub> are the wt.% of sulfur in the feed and product, respectively.

The HDN rate constant, K<sub>HDN</sub>, is determined based on first-order kinetics; that is,

$$K_{HDN} = LHSV \ln \frac{N_f}{N_p}$$

wherein N<sub>f</sub> and N<sub>p</sub> are the wppm of nitrogen in the feed and product, respectively.

In all of these experiments, the results obtained from the catalysts of this invention were compared to result obtained from commercial hydrotreating catalysts whose properties will be given in the following examples.

The catalysts prepared from metal amine metallate precursors were sulfided ex situ in a fixed-bed reactor. Typically, the sulfiding is carried out as follows: The catalyst was heated under flowing nitrogen for one hour to 370° C., held at 370° C. for one hour, then sulfided with a flowing 10% H<sub>2</sub>S-in-H<sub>2</sub> gas mixture for 10 minutes to 400° C. and held at 400° C. for two hours.

This was followed by cooling the reactor under H<sub>2</sub>S/H<sub>2</sub> to 100° C. The flow of H<sub>2</sub>S/H<sub>2</sub> was then terminated and nitrogen was introduced to flush out any remaining H<sub>2</sub>S/H<sub>2</sub>. The reactor was allowed to cool down to room temperature.

The catalysts prepared from metal amine thiometallate precursors were typically sulfided as follows: The catalyst were loaded in a fixed bed reactor. The reactor was then purged with nitrogen at 100° C. for one hour. A 10% H<sub>2</sub>S-in-H<sub>2</sub> gas mixture was then introduced to the reactor and the reactor was heated to 325° C. and held at this temperature for three hours. The reactor was then cooled to 100° C. at which point the H<sub>2</sub>S/H<sub>2</sub> flow was terminated and nitrogen was introduced. The catalyst was discharged from the reactor once the reactor was cooled down to room temperature.

The commercial catalyst was sulfided as follows: The catalyst was charged in a fixed bed reactor which was heated under nitrogen to 100° C. and held at 100° C. for one hour. A 10% H<sub>2</sub>S-in-H<sub>2</sub> gas mixture was then introduced. The reactor temperature was raised to 350° C. and held at 360° C. for one hour. Subsequently, the reactor was cooled down to 100° C. and the following gas was switched from H<sub>2</sub>S/H<sub>2</sub> to N<sub>2</sub>. The cooling was continued under N<sub>2</sub> until room temperature was reached.

## EXAMPLE 1

This example demonstrates an unexpected synergism when a metal amine molybdate-derived catalyst is placed downstream of a conventional catalyst in a stacked bed. Specifically, the catalysts used were commercial KF-742 and bulk NiMnMo sulfide prepared from the precursor Ni<sub>0.5</sub>Mn<sub>0.5</sub>(en)<sub>3</sub>MoO<sub>4</sub>. Each catalyst occupies 50% of the bed volume. KF-742 is a conventional commercial catalyst available from Ketjen. Its composition is: Mo wt. % = 11.6 and Co wt. % = 3.01, both on an elemental metal basis. This catalyst is supported on γ-Al<sub>2</sub>O<sub>3</sub> and has a BET surface area of 225 m<sup>2</sup>/g and a pore volume of 0.44 cc/g.

Shown in Table 2 is a comparison of the performances of stacked- and single-catalyst beds with Feedstock A. The volumetric activities shown in the Table were calculated based on data obtained over an on-oil period of 190 hours. The designation KF-742/NiMnMO indicates the KF-742-followed-by-NiMnMo configuration.

TABLE 2

| Catalyst Bed                      | Comparison of Stacked and Single-Catalyst Beds |                  |
|-----------------------------------|------------------------------------------------|------------------|
|                                   | k <sub>HDN</sub>                               | k <sub>HDS</sub> |
| KF-742/NiMnMo                     | 0.71                                           | 10.5             |
| KF-742                            | 0.33                                           | 7.8              |
| NiMnMo                            | 0.48                                           | 4.3              |
| Weighted Sum of KF-742 and NiMnMo | 0.41                                           | 6.1              |

As can be seen from the table, the NiMnMo and KF-742 catalysts, when used together in a stacked bed,

offer higher HDS and HDN activities than either catalyst alone. The synergism can be clearly seen by the observation that the two catalysts in the stacked bed performs better than would be expected from a weighted sum of the individual catalysts.

It is worthwhile to point out that NiMnMo itself is a relatively poor HDS catalyst. The presence of KF-742 in the upstream zone significantly improves HDS efficiency of bulk NiMnMo sulfide.

#### EXAMPLE 2

This example shows that the reverse configuration, NiMnMo-followed-by-KF742, also shows an synergism between the two catalysts. The test conditions and feedstock are the same as those employed in Example 1. The results are set forth in Table 3 below.

TABLE 3

| Catalyst Bed                      | $k_{HDN}$ | $k_{HDS}$ |
|-----------------------------------|-----------|-----------|
| NiMnMo/KF-742                     | 0.55      | 6.6       |
| KF-742                            | 0.33      | 7.8       |
| NiMnMo                            | 0.48      | 4.3       |
| Weighted Sum of KF-742 and NiMnMo | 0.41      | 6.1       |

A perusal of Tables 2 and 3 shows that with the catalyst systems (commercial and metal amine metallates/-thiometallates catalysts) of this invention, there is a pronounced effect of stacking order; the benefit of stacking KF-742 upstream of NiMnMo is greater than that of reverse stacking.

#### EXAMPLE 3

In this example, comparative experiments were done with Feedstock B under the conditions identical to those used in Example 1. The NiMnMo sulfide catalyst was not tested singly because one can tell whether there is a synergism by comparing the HDS activities of different catalyst beds. Table 4 summarizes the results.

TABLE 4

| Catalyst Bed  | $k_{HDN}$ | $k_{HDS}$ |
|---------------|-----------|-----------|
| KF-742/NiMnMo | 1.6       | 165       |
| NiMnMo/KF-742 | 1.34      | 96.3      |
| KF-742        | 0.74      | 120       |

As can be seen, the KF-742-followed-by-NiMnMo configuration shows a much higher HDS activity than KF-742 alone, despite the fact that NiMnMo is a much poorer HDS catalyst than KF-742. This again demonstrates the synergism of the stacked bed. The KF-742-followed-by-NiMnMo configuration is more effective than the reverse configuration. Once again, one sees a strong effect of stacking order with the catalyst systems of this invention. This effect is intrinsic to the present stacked-bed catalyst system, as evidenced by the following example.

#### EXAMPLE 4

These experiments compared two stacked beds comprising commercial CoMo (KF-742) and NiMo (KF-840) catalysts at 50/50 volume ratio. KF-840 is a conventional commercial catalyst available from Ketjen. Its composition is: Mo wt. % = 13.6 and Ni wt.

65

% = 2.96, both on an elemental metal basis. This catalyst is supported on  $\gamma$ -Al<sub>2</sub>O<sub>3</sub> and has a BET surface area of 162 m<sup>2</sup>/g and a pore volume of 0.35 cc/g. With Feedstock A, the following results were obtained, Table 5.

5

TABLE 5

| Catalyst Bed  | Stacked Beds Containing Commercial Catalysts |           |
|---------------|----------------------------------------------|-----------|
|               | $k_{HDN}$                                    | $k_{HDS}$ |
| KF-840/KF-742 | 0.48                                         | 7.7       |
| KF-742/KF-840 | 0.49                                         | 7.8       |

One can see that when the stacked bed contains only commercial catalysts, there is very little effect of stacking order.

What is claimed is:

1. A process for hydrotreating a hydrocarbonaceous feed, which process comprises:

(a) contacting the feed in a first catalyst zone at a temperature from about 200° C. to about 450° C., in the presence of hydrogen and a catalyst comprised of at least one metal selected from Group VIB and at least one metal selected from Group VIII of the Periodic Table of the Elements on an inorganic oxide support material; and

(b) contacting the treated feedstream from said first catalyst zone in a second catalyst zone at a temperature from about 200° C. to about 450° C., in the presence of hydrogen and a catalyst represented by the formula MM'<sub>a</sub>S<sub>x</sub> where M is Cr or one or more divalent promoter metals selected from the group consisting of Mn, Fe, Co, Ni, Cu, and Zn; M' is one or both of Mo and W; x is 0.5 to 9, and a = 1 when one of the metals represented by M is not Cr, and 1 < a ≤ 1.5 when one of the metals represented by M is Cr, wherein said catalyst is derived from a precursor selected from the formula:



where M is Cr, or one or more divalent promoter metals selected from the group consisting of Mn, Fe, Co, Ni, Cu, and Zn; L is one or more neutral, nitrogen-containing ligands at least one of which is a chelating polydentate ligand; 0 ≤ y ≤ 1; A is O or S; and a is as defined above.

2. The process of claim 1 wherein the Group VIB metal of the catalyst of the first catalyst zone is Mo, the Group VIII metal is one or both of Co and Ni, and the support material is alumina.

3. The process of claim 2 wherein M is selected from the group consisting of (a) Fe, Ni, Co and mixtures thereof and (b) mixtures of (a) with Zn, Cu, Mn and mixtures thereof.

4. The process of claim 3 wherein ligand L is selected from the group consisting of alkylamines, aryl amines, nitrogen heterocycles and mixtures thereof.

5. The process of claim 4 wherein ligand L has a total denticity of six.

6. The process of claim 5 wherein ligand L is two or three bidentate ligands.

7. The process of claim 6 wherein said tridentate and bidentate ligands are diethylenetriamine and ethylenediamine, respectively.

\* \* \* \* \*